

1

3,457,329

**INERT SIMULANT COMPOSITION FOR A PLASTIC BONDED EXPLOSIVE**

Wallace E. Silver and Jack Sherman, China Lake, Calif., assignors to the United States of America as represented by the Secretary of the Navy  
No Drawing. Filed Feb. 21, 1968, Ser. No. 707,924  
Int. Cl. C08f 29/20

U.S. Cl. 260—857

2 Claims

**ABSTRACT OF THE DISCLOSURE**

An inert simulant formulation for a high explosive composition which has the density, thermal conductivity, and thermal coefficient of expansion of the duplicated explosive and also possesses equivalent physical strength, rigidity under stress, and machinability. This formulation provides inexpensive and safe testing of mock missiles and rocket warheads and other components utilizing high explosives.

**Background of the invention**

The present invention is for an inert simulant composition for a high explosive.

In the field of explosives inert simulants or duplications thereof having the necessary characteristics for their practical use in mock warheads and similar missile components using high explosives are not known. A few compositions duplicating only one or two properties of the explosive were found but proved unsuccessful because density was the property most frequently simulated. A typical explosive simulant consisting of castor wax, ferrous oxide, calcium sulfate and wood rosin simulated only the pressed density and had the great drawbacks of melting at 187° F. Any effective valuation of aerodynamic heating effects on a mock missile war head containing this composition was precluded.

**Summary of the invention**

This invention is for an inert simulant composition for plastic bonded explosives which comprises a mixture of polytetrafluoroethylene (sold under the trade name "Teflon"), a linear polyamide (sold under the trade name "Zytel") and pentaerythritol. It duplicates the linear coefficient of thermal expansion and thermal conductivity of a plastic bonded explosive in addition to density and is also of comparable strength, easily bonded to other surfaces and readily machinable. Accordingly, this invention solved the longstanding need for an inert simulant composition possessed of sufficient of the characteristics of high explosives for use in effectively evaluating mock missile warheads and other devices which contain or use high explosives. This invention also provides an economical, practical and safe simulant for development and testing situations involving high explosive.

**Description of the invention**

In accordance with the present invention a pressable simulant composition for the plastic-bonded explosive used in a modern missile warhead was prepared. It was necessary that the simulant formulation have the following physical properties possessed by the explosive:

- (1) Density,  $1.700 \pm 0.010$  gms./cc.
- (2) Linear Coefficient of Thermal Expansion in the temperature range of  $-70^\circ$  C. to  $0^\circ$  C.,  $5 \pm 0.5 \times 10^{-5}$  in./in.-° C.
- (3) Thermal Conductivity,  $0.2 \pm 0.05$  B.t.u.-ft./hr.-° F.-ft.<sup>2</sup>.

2

The composition by weight percent which most closely simulated the plastic-bonded explosive is as follows:

|   | Ingredients:                     | Percent by weight |
|---|----------------------------------|-------------------|
| 5 | Powdered polytetrafluoroethylene | 69.8              |
|   | Powered linear polyamide         | 3.5               |
|   | Pentaerythritol                  | 26.7              |

The polytetrafluoroethylene used in this application is sold under the trademark "Teflon" and is described in United States Patent No. 2,230,654. It has a density of 2.1—2.2 gms./cc., linear coefficient of thermal expansion ( $-70^\circ$  C. to  $0^\circ$  C.)  $7.2 \times 10^{-5}$  in./in.-° C., and thermal stability of 0.14 B.t.u.-ft./hr.-° F.-ft.<sup>2</sup>. The linear polyamide sold under the trademark "Zytel" is a nylon resin of the general type described in United States Patents 2,071,250, 2,071,254 and 2,130,948. The linear polyamide used herein has a density of 1.1 gms./cc., a linear coefficient of thermal expansion ( $-70^\circ$  C. to  $0^\circ$  C.)  $12.3 \times 10^{-5}$  in./in.-° C., and thermal conductivity of 0.16 B.t.u.-ft./hr.-° F.-ft.<sup>2</sup>.

To make a fifty pound batch of the inert simulant, 1.75 lbs of "Zytel" 63 granular (soluble grade), and 54 lbs. of methanol were placed in a forty gallon slurry kettle. Water at 125° F. was turned on in the kettle jacket and the mixture stirred moderately (100 r.p.m.) until all the "Zytel" 63 was dissolved (60—120 minutes). Care should be taken not to exceed 115° F. fluid temperature inside the kettle. When the "Zytel" is completely dissolved, the stirring rate should be increased to 200 r.p.m. and first, 34.9 lbs. of powdered Teflon, then 13.35 lbs. of pentaerythritol should be gradually added by hand. Stirring should be continued at 200 r.p.m. for another 15 minutes to completely disperse both the Teflon and the pentaerythritol. When the complete dispersion in the lacquer has taken place, increase the stirring rate to 400 r.p.m. At this point, the mixture is water quenched, and the "Zytel" is released from solution with the methanol coating the pentaerythritol, while the methanol is drawn off in solution with the quench water. A large quench of 75 to 100 lbs. of 80° F.—85° F. water is added to initiate break-up of the mix into small particles. Stirring is continued at approximately 400 r.p.m. while adding the 80° F.—85° F. water as a constant rate until the kettle volume is filled. At this point, the proper particle size is achieved. The jacket is then drained of warm water, and 75° F.—80° F. cold water is added through the jacket to cool the mix. Stirring is stopped, the cold water is turned off, and the particles are allowed to settle. The supernatant liquid is then decanted off, and the remaining water-simulant mixture is manually withdrawn from the kettle. The mixture is filtered for several hours to remove additional liquid, and then oven dried overnight at 110° F. in flat trays. The dried material should possess the following particle size distribution: 10% will remain in a 5 mesh screen and less than 5% will pass through a 40 mesh screen.

The composition contained about 69.8% by weight Teflon, 3.5% by weight "Zytel" and 26.7% by weight pentaerythritol. A tabulation of the physical properties for the plastic bonded explosive and its inert simulant determined by using duplicate samples are listed below:

| Physical properties                     | Inert simulant                            | Plastic-bonded explosive                  |
|-----------------------------------------|-------------------------------------------|-------------------------------------------|
| 65 Density                              | 1.707 gms./cc.                            | 1.700 gms./cc.                            |
| Linear coefficient of thermal expansion | $4.9 \times 10^{-5}$ in./in.-° C.         | $5.4 \times 10^{-5}$ in./in.-° C.         |
| ( $-70^\circ$ C. to $0^\circ$ C.)       |                                           |                                           |
| Thermal conductivity                    | 0.21 B.t.u.-ft./hr.-° F.-ft. <sup>2</sup> | 0.19 B.t.u.-ft./hr.-° F.-ft. <sup>2</sup> |

70 This composition is pressable and is presently being successfully used for mock warhead configurations in several missile programs and to simulate the explosive charge of

various bombs which are used in conjunction with other well developed rocket programs.

Obviously many modifications and variations of the present invention are possible in the light of the above teachings. It is therefore to be understood that within the scope of the appended claims the invention may be practiced otherwise than as specifically described.

The invention described herein may be manufactured and used by or for the Government of the United States of America for governmental purposes without the payment of any royalties thereon or therefor.

What is claimed is:

1. An inert simulant formulation for high explosive compositions comprising an admixture of about 70 percent by weight polytetrafluoroethylene, about 27 percent by weight pentaerythritol and about  $4 \pm 0.5$  percent by weight linear polyamide to simulate a density from  $1.700 \pm 0.110$  gms./cc., thermal conductivity from  $0.2 \pm 0.05$  B.t.u.-ft./hr.-°F.-ft.<sup>2</sup>, and thermal coefficient of expansion in the temperature range of  $-70^\circ$  C. to  $0^\circ$  C.,  $5 \pm 0.5 \times 10^{-5}$  in./in.-°C. of said explosive composition.

2. An inert simulant formulation for a plastic-bonded explosive consisting of the following:

| Ingredients:            | Percent by weight |
|-------------------------|-------------------|
| Polytetrafluoroethylene | 69.8              |
| Pentaerythritol         | 26.7              |
| Linear polyamide        | 3.5               |

#### References Cited

##### UNITED STATES PATENTS

|    |           |         |          |           |
|----|-----------|---------|----------|-----------|
| 10 | 3,018,203 | 1/1962  | Guth     | 149-45 X  |
|    | 3,108,917 | 10/1963 | McIrvine | 149-105 X |
|    | 3,375,122 | 3/1968  | Roth     | 106-204   |

15 BENJAMIN R. PADGETT, Primary Examiner

S. J. LECHERT, Assistant Examiner

U.S. Cl. X.R.

149-92, 109; 260-33.4